

[54] **PROCESS FOR PRODUCING INGOTS BY ELECTRIC RESISTANCE MELTING PARTICULATE METAL UNDER SLAG**

[75] Inventors: **Paolo Bianchi; Aldo Ramacciotti; Eugenio Repetto**, all of Rome, Italy

[73] Assignee: **Centro Sperimentale Metallurgico S.p.A.**, Rome, Italy

[22] Filed: **Nov. 27, 1973**

[21] Appl. No.: **419,380**

[30] **Foreign Application Priority Data**

Dec. 6, 1972 Italy ..... 54535/72

[52] U.S. Cl. .... **75/10 C; 13/9; 75/10 R; 164/52**

[51] Int. Cl. .... **C22d 7/00; H05b 7/18; B22d 27/02**

[58] **Field of Search** ..... 75/10-12, 84; 164/50, 52, 250, 252; 13/9

[56] **References Cited**

UNITED STATES PATENTS

|           |         |              |         |
|-----------|---------|--------------|---------|
| 2,541,764 | 2/1951  | Herres.....  | 75/10 R |
| 2,782,245 | 2/1957  | Preston..... | 164/252 |
| 2,813,921 | 11/1957 | Vordahl..... | 75/10 R |
| 3,234,608 | 2/1966  | Peras.....   | 75/10 R |

Primary Examiner—Peter D. Rosenberg  
Attorney, Agent, or Firm—Young & Thompson

[57]

## ABSTRACT

A process for producing metal alloys in the form of large-size ingots, by melting under electro-conductive slag, wherein the material forming the alloy is partly supplied as solid metal and partly as metal in powder, granules or pellets, for conciseness called "particulate metal" comprising the sequential operations of:

- introducing into a mold, the bottom of which is made of electro-conductive material, a consumable-electrode unit, until contacts the slag;
- partially filling with said particulate metal a zone or recess provided inside said electrode unit at its end contacting the slag, closed at its bottom end by a bottom wall, and at its top by a feeding plate for the powder metal;
- establishing in said zone a controlled atmosphere by a gas circulation;
- increasing the temperature until obtaining the gradual melting of said bottom wall and the gradual simultaneous sintering of the particulate metal in said zone until forming a sintered layer having a thickness sufficient to support the weight of the superposed particulate metal;
- melting the so obtained composite electrode comprising both the electrode unit and the particulate metal continuously fed to the melting zone.

10 Claims, 1 Drawing Figure



PATENTED SEP 16 1975

3,905,803



**PROCESS FOR PRODUCING INGOTS BY  
ELECTRIC RESISTANCE MELTING  
PARTICULATE METAL UNDER SLAG**

The present invention relates to a process for manufacturing metal alloys, and more precisely, a process for manufacturing metal alloys in the form of large-size ingots, carrying out the melting operation under electrically conductive slag.

Certain processes for melting and re-melting under electrically conductive slag (processes hereinafter called ESR) are known, in some of said processes, particularly, the metals and the other elements forming the alloy being supplied to the melting zone, more or less continuously in the form of suitably mixed particles of alloys or of metals. According to one of these processes, a metal strip is used which is continuously shaped to a small-diameter tube, immediately above the ingot mold where the melting process is being carried out; this tube, besides serving the function of supplying the metal to the alloy, serves also the function of electrode and of conveyor device for the metal particles which, introduced into the tube at its top, moves freely throughout the length thereof, so as to drop continuously in the hottest zone of the liquid metal pool, and precisely under the end of the electrode. The main advantages which theoretically can be obtained by this process consist in that it is possible to control at each moment the composition of the produced ingot by changing the feeding rate of speed of the particles and of the metal electrode; also, a product particularly physically and chemically homogeneous is obtained, at least theoretically.

The actual drawbacks are due: to the size of the apparatus for forming the strip into a tube, which does not allow the simultaneous utilization of more than two or three electrodes, thus preventing the suitably rapid manufacture of big ingots; and to the rather frequent occurrence of clogging of the electrode duct by the particles, due to the small diametrical dimensions of the tube and to the slowness of the process. These drawbacks prevent practically the composition of the ingot from being controlled; in fact if the electrode tube is clogged by the particles, it is impossible to continuously adjust the composition of the produced ingot, and moreover, due to the effect of the sudden change of the selected ratio between the metal as supplied by the particles as caused by the possible clogging and the metal as supplied by the electrode, said composition has no longer the desired features of constant composition and homogeneity; furthermore, due to the slowness of the process it is impossible to obviate immediately the formation of clogs, as their effects are not immediately detectable, with the consequence that the zone showing a different analysis from the optimum will greatly enlarge.

It is to be noted, moreover, that by the process known under the ESR name it has been impossible, hitherto, to obtain ingots weighing more than a few tons, if metal powders are used, and weighing some tens of tons if an ingot is used as electrode. However, in certain sectors of the industry, for instance in the manufacture of rotors for big alternators or turbines, particularly felt is the need of having available remarkably heavy ingots, of up to some hundreds of tons, with an extremely closely controlled composition, and free from holes, inclusions, segregations, etc. Such a kind of ingot, as regards the characteristics of physical and

chemical homogeneity, can be hardly obtained by the conventional methods of melting in a furnace and teeming into an ingot mold; however, it might be obtained with an ESR process if the technical limitations concerning the weight of the so obtained ingots were not present.

A first attempt to solve this problem and to meet a very important requirement has been made by proposing a process including sequentially the operative stages both of the conventional method of ingot casting and of the ESR process. This method consists in conventionally casting an ingot having the required weight, in removing the entire inner part along the longitudinal axis which is that generally higher in physical and chemical defects, and in filling the so produced recess, by a process according to the ESR techniques. This proposal appears not to have been accepted as the ingot obtained according to this teaching has an outer zone which is not free from any of the characteristic defects of the big castings, namely stratifications of composition and physical defects, an inner zone with optimum chemical and physical characteristics, and an intermediate zone between the other two zones having intermediate physical and chemical characteristics. These differences of composition and of physical characteristics in the radial direction and the presence in the outermost layer, the most stressed, of most of the physical and chemical defects have brought the art to consider such an ingot unsuitable for the manufacture of large-sized pieces (rotors for turbines, etc.).

The purpose of this invention is to eliminate the cited drawbacks, connected with the known ESR processes using metal particles, and allowing one to overcome the problem of the low limits of weight in the produced ingots so as to allow ingots to be manufactured with uniform and controlled composition, free from the cited physical drawbacks and having a weight of some hundreds of tons.

According to the present invention a process is provided for the manufacture of metal alloys in the form of large-size ingots, by melting under electro-conductive slag, wherein the material forming the alloy is supplied in part in the form of solid metal and in part under the form of particulate metal, i.e., powder or grains or pellets, wherein with the term "particulate metal" includes one or more metal elements or alloys, suitably mixed, said process being characterized by the combination of the following steps:

- a. introducing into a mold having its bottom made of electro-conductive material a consumable electrode unit until it contacts the slag;
- b. filling partially with said particulate material a zone located inside said electrode unit at the tip thereof contacting the slag, said zone being delimited at its bottom by a bottom wall closing said end and at its top by a feeding plate for the metal particles;
- c. establishing in said zone a controlled atmosphere by gas circulation;
- d. increasing the temperature until obtaining the gradual melting of said bottom wall and the gradual simultaneous sintering of the metal particles in said zone until forming a layer having a thickness sufficient to support the weight of the superposed column of the particulate material;
- e. melting the composite electrode so obtained, comprising both the electrode unit and the metal particles continuously fed to the melting zone.

The equipment used according to this invention for carrying out this process includes a consumable electrode system which is characterized by one or more cylindrical metal tubes, preferably one to four, for feeding the metal, each with a diameter variable from 20 to 90 percent of the diameter of the ingot to be produced, said tubes being extendable by means of welding of further portions of tube to that, or to those, which is, or are being melted, throughout the duration of the melting process.

The present invention will be now described with particular reference to the attached drawing showing by way of non-limitative example one preferred embodiment of the equipment according to this invention, using a single electrode.

Particularly, in the attached drawing the FIGURE shows a sectional vertical view, of a scheme of a facility for the manufacture of ingots by the process according to this invention.

With reference to the FIGURE, therein are shown a mold 1, of conventional ESR type, inside of which has been shown the liquid metal pool, and the superposed layer 6 of molten slag, into which is immersed the lower tip of a metal tubular electrode 2 supported and guided by technologically suitable means, of a substantially conventional kind.

It is to be noted that said tubular electrode 2 is provided in its lower part with a recess or zone 5 downward delimited, at the start of the re-melting, by a bottom wall 3 at least 35 mm thick, closing the lower end of the electrode 2, and at its top, by a feeding plate 4 which will be described in greater detail hereinafter. Inside the pipe 5 have been shown the layer 7 of the already sintered metal particles under the superposed column of metal particles 10 which drops downwards in the recess 5, passing through the duct 8 and the hole or holes 11 of the plate 4.

As far as the course of the process according to this invention is concerned, initially the lower tip of the electrode 2 submerged into the slag is closed by a metal bottom wall 3 fixed to the walls of the electrode 2 inside of which is introduced the metal particles by a feeding plate 4. This plate and the cited bottom wall 3 define a recess 5 which is thus partially filled with the metal particles. Inside said recess a controlled atmosphere will be established by a gas circulation, for instance using an inert gas such as argon. Then through each electrode an alternating or direct current (20 to 100 V and 5,000 to 60,000 A) is caused to pass through the circuit the electrodes of which are the metal tube and the mold. This current, due to the Joule effect, develops a large amount of heat within the slag 6 under the electrode 2, causing thus the gradual melting of the bottom wall 3 and simultaneously the gradual sintering of an ever increasing layer 7 of metal particles, inside said recess 5. When the bottom wall is entirely melted, the sintered layer 7 has still a thickness sufficient to support the superposed particle column 10, which is still incoherent. Said layer 7 serves now the function of bottom wall and the melting process of the sintered layer and of simultaneous sintering of a layer of metal particles assumes a stable operative condition.

The metal tube 2 serving the function of an electrode will be downwards moved at a rate of speed comprised between 1 and 10 cm per min., and the particulate metal is fed so as to keep almost constant its volume within the recess 5.

The feeding plate 4 consists of a disk made either of metal or of any other suitable material, having a diameter a little less than the internal diameter of the electrode 2; said plate is transected by one or more holes 11, provided with delivery valves, into which are inserted the duct and the feeding components 8 for the metal particules, and by one or more holes 12 into which are inserted the duct or ducts 9 for feeding the gas for establishing the controlled atmosphere ambient.

10 This plate is supported by means different from said feeding ducts for the powder and for the gas, and is located in fixed position with respect to the mouth of the mold 1, or inside the mold itself, and in this case it will be slowly upwards moved in order to maintain constant its distance from the molten metal pool. The feeding ducts for the particules and for the gas are independent from the electrode, said ducts can be disconnected from the plate and removed from the electrode in order to allow the coupling of the operating electrode to the subsequent lengths of tube.

15 The metal which will be supplied inside the cylindrical tube 2 and which fills the recess 5 can be supplied, as afore said, in the form of powder, of granules or of pellets.

20 If only powders are used, the most suitable grain sizes are the finest available on the market, and the lower limit of size is determined only by the cost of the powders themselves.

25 It is possible, however, to use coarse powders, with a maximum grain size of 4 mm, and in this case it is necessary to mix said coarse powders with finer powders in the percent of at least 20 percent by weight so as to obtain for the mixture an apparent bulk density of at least 2.7 grams/cc.

30 On the otherhand, if granules or pellets are to be used it will be necessary to mix therewith at least 20 percent by weight of a mixture of powders and small granules, the size of which is between 0.01 and 4 mm, so as to obtain a final mixture having an apparent bulk density of at least 2.6 grams/cc.

35 In the light of the practical and theoretical information available before the experiments which led to this invention, the solution here proposed for the technical problem of the production of big ingots with the ESR technique appeared to be doubtfully applicable. In fact, a set of considerations as to the sintering rates of the non compressed metal particles, as to the melting rate which must be rather high in order to allow big ingots to be manufactured with industrially acceptable speed, as to the mechanical resistance of the sintered metal products at high temperatures, and as to the thermal and electrical conductivity of the metal powders in incoherent mass, caused the art to consider the process as above described to be hardly capable of being practiced.

40 The subsequent tests, on the contrary, demonstrated that other theoretically more effective solutions were not capable of being practiced for either economical or technical reasons, while surprisingly this invention could be successfully applied, as is clearly shown by the following example disclosed for illustrative and non-limitative purposes.

45 In a water-cooled metal mold having a diameter of 800 mm, have been placed 350 kgs of slag having the composition by weight as follows:

CaF<sub>2</sub> 40%; Al<sub>2</sub>O<sub>3</sub> 30%; CaO 24%; MgO 6%

Into said slag a hollow metal cylinder the outer diameter of which was 500 mm, with a wall 15 mm thick, was immersed for 15  $\div$  20 mm. The immersed end of said cylinder was closed by a bottom plate 100 mm thick. Over said bottom plate, under circulation of argon, a layer of metal powder has been accumulated, with a maximum grain size corresponding to 0.2 mm, and with a height varying from 400 to 500 mm. The analysis of the steel used for the tube, the bottom and the powder was:

C 0.25; Mn 0.50; P 0.01; S 0.009; Si 0.25; Ni 3; Cr 0.30; O<sub>2</sub> 60 ppm

the balance consisting of Fe and minor impurities.

The used alternating current at 50 Hz, had 50 V and 20,000 A.

In steady condition of operation, the temperature of the slag was 1650  $\div$  1,700°C; the downwards feed rate 20 of the electrode was about 3.3 cm/min., and the supply rate of the powder was 500 kgs/h.

After 24 hours an ingot has been obtained weighting 15 tons and having the composition as follows:

C 0.27; Mn 0.46; P 0.008; Si 0.13; Ni 30; Cr 0.30; S 25 0.008; O<sub>2</sub> 50 ppm

the balance consisting of Fe and minor impurities.

This composition appeared to be substantially constant throughout the longitudinal and transverse sections of the ingot and also the mechanical properties appeared to be uniform.

The present invention has been described with particular reference to certain specific embodiments thereof, but it is to be understood that modifications might be entered without thereby departing from the scope of the invention as defined by the appended claims.

Having thus described the present invention, what is claimed is:

1. An ESR process for producing metal alloy ingots by melting under electro-conductive slag, comprising

establishing in an electro-conductive mold a quantity of slag, introducing into said mold a hollow consumable metal electrode having a closed bottom immersed in said slag, introducing particulate metal into said hollow electrode, establishing an inert gas atmosphere in said hollow electrode, passing an electric current through said electrode and mold to melt said closed end of the electrode and to sinter said particulate metal adjacent said end of the electrode to form a sintered layer having a thickness sufficient to support the weight of the superposed particulate metal, and supplying further particulate metal to the interior of said electrode while continuing to pass said electric current thereby progressively to melt said particulate metal and said electrode and progressively to build a said ingot in said mold.

2. A process as claimed in claim 1, and feeding said electrode downwardly into said mold at a rate between 1 to 10 cm/min.

3. A process as claimed in claim 2, and welding further hollow electrodes to said hollow electrode to replace the material of the electrode consumed by melting.

4. A process as claimed in claim 1, in which said particulate material has a grain size up to 4 mm.

5. A process as claimed in claim 1, in which the bulk density of said particulate metal is at least 2.7 g/cc.

6. A process as claimed in claim 1, in which said electric current is 20 to 100 volts and 5,000 to 60,000 amperes.

7. A process as claimed in claim 1, and maintaining the end of said electrode a constant distance above the level of the metal bath that forms atop said ingot.

8. A process as claimed in claim 1, in which said electrode has a diameter from 20 percent to 90 percent the diameter of the ingot to be produced.

9. A process as claimed in claim 1, said particulate metal and electrode being steel.

10. A process as claimed in claim 1, said particulate metal and said electrode having the same composition.

\* \* \* \* \*